

# United States Patent Office

2,912,314

Patented Nov. 10, 1959

1

2,912,314

## CRACKED FUEL OILS STABILIZED WITH AMINE SALTS OF DITHIOCARBAMIC ACIDS

Henry C. Geller, Wilmington, Del., and Bernard Miller Sturgis, Pitman, N.J., assignors to E. I. du Pont de Nemours and Company, Wilmington, Del., a corporation of Delaware

No Drawing. Application May 1, 1956

Serial No. 581,845

5 Claims. (Cl. 44—72)

This invention is directed to new inhibitors in the form of amine salts of dithiocarbamic acids for fuel oils containing cracked hydrocarbons boiling in the fuel oil range, said inhibitors improving the storage properties of said fuel oils.

Commercial fuel oils, as sold for use in oil burners, furnaces, diesel engines and jet engines, are produced from straight-run hydrocarbon distillates and from petroleum crudes resulting from thermal and catalytic-cracking. Fuel oils are produced more economically and in larger volumes by thermal- and catalytic-cracking methods; increased demand for fuel oils is met largely by increased production of cracked stocks.

It is known that fuel oils consisting essentially of or containing in part cracked hydrocarbons are subject to serious discoloration and formation of insoluble sludge during storage. This pronounced instability in contrast to the comparative inertness of straight-run distillates is attributed primarily to oxidation, polymerization and condensation reactions of olefins and diolefins and of sulfur and nitrogen compounds present in the cracked (particularly catalytic-cracked) fuel oils.

In general, discolored fuel oils as hereinbefore described are objectionable to the trade as certain color standards have to be met in marketing fuel oils. Deposition of insoluble sludge in storage is particularly undesirable in that the deposits plug filter screens, orifices, nozzles, etc.

Special refining techniques for improving storage stability of fuel oils involve relatively costly operations; thus, there is a need for incorporating into said fuel oil relatively small quantities of chemicals as inhibitors against deterioration in storage.

It is an object of the present invention to provide a fuel oil containing catalytic-cracked hydrocarbons boiling in the fuel oil range stabilized against sludge formation and discoloration by incorporating into said fuel oils small quantities of a suitable additive as inhibitor.

More specifically, the present invention is directed to a fuel oil containing catalytic-cracked hydrocarbon stocks boiling in the fuel oil range, and, as an inhibitor of discoloration and sludge formation, from 0.001% to 0.5% of a fuel-soluble amine salt of a dithiocarbamic acid, said inhibitor having the formula



where  $R_1$ ,  $R_2$ ,  $R_3$ , and  $R_4$  are taken from the group consisting of alkyl radicals, cycloalkyl radicals, and alkylene radicals which together with nitrogen constitute a heterocyclic ring, there being a total of at least 5 carbon atoms attached to each nitrogen.

By fuel oils is meant those hydrocarbon fuels which are heavier than gasoline and adaptable for use in oil furnaces, diesel engines and jet engines.

In addition, by fuel oils containing cracked hydrocarbons boiling in the fuel range is meant catalytic-cracked fuel oils, or blends of straight-run fuel oil distillates and said catalytic cracked oils containing about 20% or more of said catalytic-cracked oils.

The fuel-soluble amine salts of dithiocarbamic acids of

2

the present invention are disubstituted-ammonium di-substituted-dithiocarbamates, as indicated in the formula:



5 Representative substituents of the alkyl and cycloalkyl type are: methyl, ethyl, n- and isopropyl, n-, iso- and sec.-butyl, n- and isoamyl, hexyl, cyclopentyl, cyclohexyl, cycloheptyl, octyl, decyl, dodecyl, tetradecyl, heptadecyl, octadecyl and the like.

10 When each nitrogen atom bears two such separate (i.e., monovalent) substituents, the total carbon content of the two groups should be at least 5. One of the substituents may be a methyl group; it is preferred there be at least 4 carbon atoms in each group.

15 The substituents attached to nitrogen may be divalent alkylene radicals having at least 5 carbon atoms in the divalent unit, e.g., pentamethylene and hexamethylene, which together with the nitrogen atom form a heterocyclic unit, e.g. piperidino (pentamethyleneimino), and hexamethyleneimino radicals.

20 It is convenient to name and represent the additives of this invention as "salts." It should be understood, however, that in non-polar hydrocarbon media, they may exist as hydrogen-bonded entities with little or no separation of the potentially ionic groups occurring, such as



25 The fuel-soluble amine salts of dithiocarbamic acids of this invention may be prepared by reacting one mole of carbon disulfide with two moles of a suitable secondary amine. Suitable secondary amines, which may be employed singly or as mixtures, are disubstituted ammonia molecules in which the substituents on nitrogen are alkyl, cycloalkyl, or alkylene radicals, as defined. That is, the nitrogen atom may carry two separate (monovalent) groups, which may be the same or different groups but totalling at least 5 carbon atoms; or the NH function may be part of a ring which is completed by a divalent alkylene portion having at least 5 carbon atoms in the divalent unit.

30 Specific examples of fuel-soluble amine salts of dithiocarbamic acids of this invention are: methyl-n-butylammonium methyl-n-butylthiocarbamate, ethylisopropylammonium ethylisopropylthiocarbamate, diisopropylammonium diisopropylthiocarbamate, di-n-butylammonium di-n-butylthiocarbamate, diisobutylammonium diisobutylthiocarbamate, dicyclohexylammonium dicyclohexylthiocarbamate, cyclohexylethylammonium cyclohexylethylthiocarbamate, dioctadecylammonium dioctadecylthiocarbamate, piperidinium pentamethylenedithiocarbamate. Compounds representative of the above, and similar compounds encompassed by this invention, are described in the accompanying examples illustrating the present invention.

35 The preferred compounds are: dicyclohexylammonium dicyclohexylthiocarbamate; diisopropylammonium diisopropylthiocarbamate; dibutylammonium dibutylthiocarbamate, e.g., in which n-butyl and isobutyl groups are equally present (i.e., prepared from equimolar mixture of di-n- and diisobutylamines); diamylammonium diamylthiocarbamate, e.g., as prepared from commercial mixed diamylamines.

40 The quantities of amine salts of dithiocarbamic acids selected for use in the fuel oil will depend upon the instability of the particular oil to be stabilized and the effect desired. However, it has been found that less than 0.001% by weight based on the fuel oil, is relatively ineffective. On the other hand it is seldom necessary to use more than 0.5% of the active ingredients based on

the entire weight of the fuel oil to be treated. The preferred range is 0.005 to 0.1%.

The defined stabilizers may be incorporated into the fuel oil simply by adding them to the main body of oil and stirring at ordinary temperatures. In another embodiment of the invention the stabilizer or mixture of stabilizers is incorporated into a carrier, e.g., kerosene or xylene, in high concentrations—normally about 50% by weight of the concentrate. This concentrated solution represents the commercial form of the stabilizer to be shipped to the refinery where it is added to the main body of the fuel oil to be stabilized. To prepare such concentrated solutions, amine salts of high solubility are required. The mixed salt prepared from equimolar quantities of di-n- and diisobutylamine is particularly satisfactory for this purpose.

Other valuable amine salts for this purpose are those derived from commercially available mixtures of secondary amines, such as the isomeric dibutylamines, the diamylamines, and, the "dicoco amines" which are understood to be a mixture of long chain secondary amines (di-n-C<sub>8</sub> to di-n-C<sub>18</sub>), prepared from coconut oil. The disubstituted ammonium disubstituted dithiocarbamates obtained from these mixed amines and mixtures of said mixed amines are either low melting solids or liquids having high solubility in hydrocarbons.

The dithiocarbamates of this invention which prevent color and sludge formation may be employed in conjunction with other additives for fuel oils, such as metal deactivators and dispersants for fuel oil sludge.

The following examples illustrate the invention.

#### EXAMPLE 1

Various catalytically-cracked fuel oil No. 2 distillates (A to D in the table) were inhibited against color deterioration and insoluble residue formation by adding 0.005 weight percent of amine salts of dithiocarbamic acids. The fuels were subjected to a high-temperature accelerated test wherein 600 gram samples in vented glass bottles were stored at 210° F. for 16 hours. After cooling the samples to room temperature, their NPA colors were determined and compared with the original colors according to ASTM Method D155-45T. To determine the quantity of sediment formed, each sample was filtered by suction through a tared sintered glass filter having a 1.125 inch diameter and an average pore size of 14 microns. The filter was washed with heptane, dried and weighed.

The results of these tests were as follows:

Table 1

EFFECT OF 0.005% BY WEIGHT OF AMINE SALTS OF DI-THIOCARBAMIC ACIDS ON FUEL OILS AGED AT 210° F. FOR 16 HRS.

| Test | Fuel Oil | Additive                                                 | NPA Color |       | Insoluble Residue, mg./600 g. |
|------|----------|----------------------------------------------------------|-----------|-------|-------------------------------|
|      |          |                                                          | Before    | After |                               |
| 1    | A        | None                                                     | 1.5—      | 3.5—  | 6.0                           |
| 2    | A        | diisopropylammonium diisopropylthiocarbamate.            | 1.5—      | 2—    | 2.4                           |
| 3    | B        | None                                                     | 1.5—      | 5.5—  | 5.6                           |
| 4    | B        | piperidinium pentamethyleneedithiocarbamate.             | 1.5—      | 2.5—  | 0.7                           |
| 5    | C        | None                                                     | 2—        | 7.5—  | 12.1                          |
| 6    | C        | dicyclohexylammonium dicyclohexyl-dithiocarbamate.       | 2—        | 2—    | 0.9                           |
| 7    | C        | "dicocoammonium dicoco-dithiocarbamate." <sup>1</sup>    | 2—        | 2—    | 0.6                           |
| 8    | D        | None                                                     | 1.5—      | 4—    | 30.0                          |
| 9    | D        | ethylcyclohexylammonium ethylcyclohexyl-dithiocarbamate. | 1.5—      | 1.5   | 3.8                           |

<sup>1</sup> Prepared from "dicocoamine" by reaction with carbon disulfide. "Dicocoamine" is commercially available as "Arveen 2C" and consists substantially of secondary aliphatic amines RRNH where R has the following approximate composition: n-octyl 8%, n-decyl 5%, n-dodecyl 47%, n-tetradecyl 18%, n-hexadecyl 8% and n-octadecyl 10%.

As can be seen from these results, the additives of this invention markedly improve resistance to discoloration and formation of insoluble residue of fuel oils showing varying tendencies to discolor and form sludge.

The procedure of Example 1 was repeated using 0.005% by weight of various amine salts of dithiocarbamic acids in typical samples of catalytically-cracked fuel oil No. 2 distillates, designated as fuel oils E and F in the table below. The results of these tests were as follows:

Table 2

| 15 | Test | Fuel Oil | Additive                                           | NPA Color |            | Insoluble Residue, mg./600 g. |
|----|------|----------|----------------------------------------------------|-----------|------------|-------------------------------|
|    |      |          |                                                    | Before    | After      |                               |
| 11 | 11   | E        | None                                               | 2—        | 4.5—       | 13.1                          |
| 12 | 12   | E        | dimethylammonium dimethyl dithiocarbamate.         | 2—        | 3.5—       | 25.4                          |
| 20 | 13   | E        | dicyclohexylammonium dicyclohexyl-dithiocarbamate. | 2—        | 3—         | 2.0                           |
| 25 | 14   | F        | None                                               | 2—        | 5—         | 29.6                          |
| 15 | 15   | F        | diethylammonium diethyl-dithiocarbamate.           | 2—        | 4—         | 37.5                          |
| 16 | 16   | F        | piperidinium pentamethylene dithiocarbamate.       | 2—        | (haze) 2.5 | 6.2                           |

Tests 12 and 15 illustrate compounds which are outside the scope of our invention and which are clearly ineffective stabilizers, particularly against sludge formation, of these cracked oils.

#### EXAMPLE 3

The procedure of Example 1 was repeated on samples of catalytically-cracked fuel oil No. 2 distillate containing a dialkylammonium dialkylthiocarbamate. The results obtained with 0.005% by weight of additive based on the treated fuel oil were as follows:

Table 3

| 45 | Test | Additive                                                                                                       | NPA Color |            | Insoluble Residue, mg./600 g. |
|----|------|----------------------------------------------------------------------------------------------------------------|-----------|------------|-------------------------------|
|    |      |                                                                                                                | Before    | After      |                               |
| 17 | 17   | None                                                                                                           |           |            | 35.6                          |
| 18 | 18   | dibutylammonium dibutylthiocarbamate (prepared from equimolar mixture of di-n-butylamine and diisobutylamine). | 1.5       | 3.5—<br>2— | 4.8                           |

#### EXAMPLE 4

A catalytically-cracked fuel oil was treated with 0.005 weight percent of dicyclohexylammonium dicyclohexyl-dithiocarbamate and 300 ml. samples, along with untreated samples as controls, were subjected to a low temperature aging test in vented glass bottles, at 110° F., in the dark for 15 weeks. At the end of the aging period, first the NPA color of each sample was determined at room temperature, then the sample was filtered through a sintered glass filter having a 1.25 inch disc with an average pore size of 5 microns. The original container and filter were washed with naphtha. The insoluble residue remaining in the container and filter was dissolved in 1:1 acetone-methanol solutions, and the quantity determined by airjet evaporation according to ASTM Method D525-46.

The control samples containing no added stabilizer had color ratings of 5— NPA units (i.e., red-brown), and yielded 33.7 mg. of insoluble residue per 100 ml. of fuel oil, whereas samples of fuel oil containing the dicyclohexylammonium dicyclohexylthiocarbamate had color ratings of 4.5— NPA units (i.e., light orange), and had

produced only 5.7 mg. of insoluble residue per 100 ml. of sample.

## EXAMPLE 5

A concentrate containing 50% by weight of mixed dibutylammonium dibutylthiocarbamates in kerosene was prepared directly as follows:

7.6 parts carbon disulfide were added slowly to a stirred solution of 12.9 parts of di-n-butylamine and 12.9 parts of diisobutylamine in 23.4 parts of kerosene, at 5-10° C. The addition of carbon disulfide completed, the delivery system was rinsed with 10 parts kerosene and the washings added to the reaction mass. The reaction mass was stirred for one hour at 5-10° C., was warmed briefly to 45° C., and then allowed to cool to room temperature to obtain a clear yellow liquid product containing 50% active ingredient.

Samples of this concentrate effectively stabilized catalytically-cracked fuel oil No. 2 distillates under conditions of the accelerated aging test (210° F. for 16 hours) described in Example 1.

Before being aged, all samples including the control had NPA color ratings of 1.5. After being aged, the control sample containing no added stabilizer had a color rating of 4—NPA units and yielded 43.0 mg. of insoluble residue for each 600 ml. of sample tested. The fuel oil samples containing from 0.001% to 0.1% by weight of active ingredient, had NPA color ratings of 2—after being aged, and yielded from 3.4 to 6.6 mg. of insoluble residue for 600 ml. of aged sample. Concentrates may be prepared, according to this procedure, by starting with various mixtures of isomeric dibutylamines or isomeric diamylamines. Substantially the same beneficial results are obtained on employing concentrates of these dialkylammonium dialkyldithiocarbamates as inhibitors in the 35 above example.

## EXAMPLE 6

Concentrates containing 50% by weight of dialkylammonium dialkyldithiocarbamates in xylene were prepared by reacting the following mixtures of secondary amines with carbon disulfide in the ratio of 2 moles of amine to one mole of carbon disulfide, employing the reaction conditions given in Example 5:

| Sample | Sec-Amine Mixture            | Mole Ratio of Mixture |
|--------|------------------------------|-----------------------|
| A      | methyl-n-butyl+di-n-butyl... | 1:2                   |
| B      | dicoco 1+di-n-butyl...       | 1:1                   |
| C      | diamyl 2+di-n-butyl...       | 1:3                   |

<sup>1</sup> The composition of dicocoamine is given in a footnote to Table 1, Example 1.

<sup>2</sup> Commercially available mixture of isomeric diamylamines.

Catalytically-cracked No. 2 fuel oil was inhibited against color deterioration and insoluble residue formation by adding 0.0025 weight percent active ingredient of the concentrates prepared from amine mixtures A, B and C above. The treated fuels were aged as described in Example 1. The results of the tests were as follows:

Table 4

EFFECT OF 0.0025 WT. PERCENT DITHIOCARBAMATE ON FUEL OIL AGED AT 210° F. FOR 16 HOURS

| Additive from— | NPA Color |       | Sludge, mg./600 g. |
|----------------|-----------|-------|--------------------|
|                | Before    | After |                    |
| None           | 1         | 7—    | 31.2               |
| A              | 1         | 1.5   | 3.8                |
| B              | 1         | 1.5   | 1.8                |
| C              | 1         | 1.5   | 2.9                |

## EXAMPLE 7

Concentrates, suitable for use as stabilizers for fuel oil, were prepared by mixing 25 parts of a dialkylammonium dialkyldithiocarbamate, 25 parts of kerosene and 50 parts of a kerosene solution containing 25 parts of a 50/40/10 tripolymer of octadecenyl methacrylate (technical)/styrene/beta-diethylaminoethyl methacrylate. Preparation and use in fuel oil of the tripolymer and related polymers which may also be employed in conjunction with the additives of the present invention are described in U.S. Patents 2,737,452 and 2,737,496.

For example, Blend X was prepared using di-sec-butylammonium di-sec.-butyldithiocarbamate. Blend Y was prepared using mixed dibutylammonium dibutyl-dithiocarbamates obtained by reacting an equimolar mixture of di-n-butylamine and diisobutylamine with carbon disulfide (see Example 5). These concentrates may be employed in conjunction with a metal deactivator (MDA) such as N,N'-disalicylidene-1,2-propanediamine, as shown below.

Samples of fuel oil containing catalytically-cracked hydrocarbons boiling in the fuel oil range, with and without stabilizer present, were aged according to the procedure given in Example 1 (210° F., 16 hours). Results of these tests were as follows (Table 5):

Table 5

EFFECT OF CONCENTRATES ON FUEL OIL AGED AT 210° F. FOR 16 HOURS

| Fuel Oil Additive                 | NPA Color |       | Insoluble Residue, mg./600 g. |
|-----------------------------------|-----------|-------|-------------------------------|
|                                   | Before    | After |                               |
| None                              | 2—        | 5—    | 5.8                           |
| Blend X <sup>1</sup> +0.0007% MDA | 2—        | 3—    | 0.6                           |
| Blend Y <sup>1</sup> +0.0007% MDA | 2—        | 3—    | 1.4                           |

<sup>1</sup> Blends X and Y employed in quantities sufficient to provide 0.005% by weight, based on the fuel oil, of the dithiocarbamate and of the tripolymer.

45

This data shows that the amine salts of the dithiocarbamic acids are extremely effective color stabilizers under conditions of the test in addition to effecting a high reduction in residue formation.

The present invention applies to the stabilization of cracked fuel oils, particularly those entirely composed of catalytic-cracked oil or those containing rather high proportions (at least 20%) of catalytic-cracked oil inasmuch as the catalytic-cracked fuels are notoriously subject to deterioration in storage. An outstanding advantage of this invention is that it provides cracked fuel oils having greatly improved resistance to sludge formation and having improved color stability.

We claim:

1. A fuel oil containing catalytic cracked hydrocarbon stocks boiling in the fuel oil range and from 0.001% to 0.5% of a fuel-soluble amine salt of a dithiocarbamic acid as inhibitor, said inhibitor having the formula



70  
75  
wherein R<sub>1</sub>, R<sub>2</sub>, R<sub>3</sub> and R<sub>4</sub> are taken from the group consisting of alkyl radicals, cycloalkyl radicals, and alkylene radicals which together with nitrogen constitute a heterocyclic ring, there being a total of at least 5 carbon atoms attached to each nitrogen.

2. The fuel oil of claim 1 wherein the inhibitor is dicyclohexylammonium dicyclohexylthiocarbamate.

3. The fuel oil of claim 1 wherein the inhibitor is diamylammonium diamyldithiocarbamate.

4. The fuel oil of claim 1 wherein the inhibitor is dibutylammonium dibutyldithiocarbamate.

5. The fuel oil of claim 1 wherein the inhibitor is a mixture of dibutylammonium dibutyldithiocarbamate and diamylammonium diamyldithiocarbamate.

References Cited in the file of this patent

UNITED STATES PATENTS

|              |                |                |
|--------------|----------------|----------------|
| 2,160,851    | Faust          | June 6, 1939   |
| 2,343,393    | Bergen         | Mar. 7, 1944   |
| 5 2,385,964  | Bergen         | Oct. 2, 1945   |
| 2,400,106    | Denison et al. | May 14, 1946   |
| 2,636,858    | Jones          | Apr. 28, 1953  |
| 2,716,089    | Cyphers et al. | Aug. 23, 1955  |
| 10 2,805,996 | Deger          | Sept. 10, 1957 |

UNITED STATES PATENT OFFICE  
CERTIFICATE OF CORRECTION

Patent No. 2,912,314

November 10, 1959

Henry C. Geller et al.

It is hereby certified that error appears in the printed specification of the above numbered patent requiring correction and that the said Letters Patent should read as corrected below.

Column 1, line 30, for "intertness" read -- inertness --; column 3, line 75, in the footnote to Table 1, for "7%" read -- 47% --; column 4, Table 3, under the heading "Additive", first line thereof, for "nond" read -- none ---.

Signed and sealed this 3rd day of May 1960.

(SEAL)

Attest:

KARL H. AXLINE  
Attesting Officer

ROBERT C. WATSON  
Commissioner of Patents